# EUROPEAN PATENT APPLICATION

(11) **EP 4 233 576 A1**
(43) Date of publication of application: **30.08.2023**
(21) Application number: 21885175.6
(22) Date of filing: 26.10.2021
(51) Int. Cl.: A24D 1/04, A24D 3/17, A24D 1/20, A24D 3/02

(54) **TOBACCO PRODUCT AND PLANT-FLAVORED FILTER STICK THEREOF, AND PREPARATION METHOD THEREFOR**

(30) Priority: 27.10.2020 CN 202011163680
(71) Applicant: Shanghai Huabao Biology Technology Co., Ltd., Shanghai 201800 (CN)
(72) Inventor: GAO, Xu, Shanghai 201800 (CN); SHEN, Li, Shanghai 201800 (CN); XU, Xiaodong, Shanghai 201800 (CN); LIANG, Jiasheng, Shanghai 201800 (CN); YING, Yu, Shanghai 201800 (CN); CAO, Tongtong, Shanghai 201800 (CN); FU, Yuanfeng, Shanghai 201800 (CN); YAO, Jianwen, Shanghai 201800 (CN); SUN, Wenxuan, Shanghai 201800 (CN)
(74) Representative: HGF
(86) International application number: PCT/CN2021/126504
(87) International publication number: WO 2022/089448

(57) **Abstract**

A tobacco product, a plant-flavored filter stick, and a preparation method therefor, wherein the plant-flavored filter stick is implemented to be provided with pores penetrating the two ends of a filter tip section (30); and the plant-flavored filter stick comprises 4-5 parts by weight of a plant raw material powder with a fragrance, 4-6 parts by weight of a smoke agent, 4-6 parts by weight of a binder, and 4-6 parts by weight of water, and is capable of achieving the fragrance enhancement of a tobacco product. The fragrance enhancement of the tobacco product is achieved by means of the natural fragrance of the filter stick itself, and the fragrance emitted by a fragrance enhancing material added to the filter stick in the plant-flavored filter stick. In addition, the plant-flavored filter stick can avoid the escape and pyrolysis of the fragrance enhancing material during the storage and smoking process of the tobacco product.

## Description

### Cross-Reference to Related Applications

The present disclosure claims priority to Chinese Patent Application No. 202011163680.0, entitled "Tobacco Product and Plant-Flavored Filter Stick Thereof, and Preparation Method Therefor", filed with the Chinese Patent Office on October 27, 2020, the contents of which are incorporated herein by reference in entirety.

### Technical Field

The present disclosure relates to the field of cigarette, and particularly to a tobacco product and a plant-flavored filter stick thereof, and a preparation method therefor.

### Background Art

With the increasing call for smoke banning internationally and as cigarette consumers increasingly value their own health, low-tar and low-harm cigarettes have become the new normal in the tobacco market. However, the reduction of tar and harm inevitably leads to the loss of cigarette aroma and a deterioration in comfort. While adding flavor to the cigarette can support and supplement cigarette aroma, remove and cover up miscellaneous gases, thereby not only reducing the irritation of cigarettes, but also endowing the cigarette products with elegant characteristic aroma, such that the personalized style of cigarette products is highlighted. The development and application of adding flavor to the cigarette is becoming one of the key technologies to maintain the aroma of cigarettes in the work of reducing harm and tar.

Currently, cigarette aroma addition mainly includes two methods: cigarette component aroma addition and cigarette accessory aroma addition. Because the amount of aroma added to cigarettes by the cigarette component aroma addition method is limited, and cigarette accessory aroma addition can make up for the shortcomings of insufficient aroma addition amount by the cigarette component aroma addition, most of the existing research and development of cigarettes are carried out towards the method of cigarette accessory aroma addition.

Cigarette accessory aroma addition is mainly achieved through the addition of aroma to cigarette paper, liner paper, tipping paper, and filter stick. However, cigarette paper itself burns, liner paper and tipping paper have defects like limitations on aroma addition amount and short aroma retention time. Therefore, cigarette accessory aroma addition mainly is aroma addition to filter stick. Aroma addition to cigarette filter stick mainly includes aroma addition by bubbles, tows and particles. Aroma addition by bubbles has high cost and is limited by the addition of oily flavor substances. Aroma addition by tows and particles have problems such as low adsorption of flavor substances and uneven aroma addition.

### Summary

The present disclosure provides a tobacco product and a plant-flavored filter stick thereof, and a preparation method therefor, wherein the plant-flavored filter stick utilizes the natural aroma of the filter stick itself and the aroma released by flavor-enhancing substances added to the filter stick to enhance the aroma of the tobacco product.

The present disclosure provides a tobacco product and a plant-flavored filter stick thereof, and a preparation method therefor, wherein the plant-flavored filter stick can avoid the loss and thermal degradation (the escape and pyrolysis) of flavor-enhancing substances during the storage and burning-smoking process of the tobacco product.

The present disclosure provides a tobacco product and a plant-flavored filter stick thereof, and a preparation method therefor, wherein the plant-flavored filter stick can reduce a burning sensation felt by user when smoking.

The present disclosure provides a plant-flavored filter stick, wherein the plant-flavored filter stick can be implemented as a filter stick having a gas hole passing through two ends of the filter segment (filter tip segment), and the plant-flavored filter stick can include:
4-5 parts by weight of plant raw material powder with aroma;
4-6 parts by weight of smoking agent;
4-6 parts by weight of adhesive; and
4-6 parts by weight of water.

According to one example of the present disclosure, the plant powder can include cultivated plants and wild plants with aroma.

According to one example of the present disclosure, the plant-flavored filter stick can include a predetermined amount of essence solidified on the plant-flavored filter stick.

According to one example of the present disclosure, the essence can include at least one of water-soluble essence, oil-soluble essence and microencapsulated essence.

According to one example of the present disclosure, the solvent of the oil-soluble essence can be preferably selected from the group consisting of medium-chain triglyceride, glycerol triacetate, and triethyl citrate.

According to some embodiments of the present disclosure, the present disclosure provides a tobacco product, the tobacco product can include a smoking segment, a cooling segment and a filter segment, wherein the smoking segment and the filter segment can be provided at two ends of the cooling segment, respectively. The filter segment can be implemented as the plant-flavored filter stick according to any one of claims 1-5.

According to one example of the present disclosure, the cooling segment is implemented as a plant element with porous structure penetrating through the cooling segment.

According to some embodiments of the present disclosure, the present disclosure provides a preparation method of the plant-flavored filter stick, wherein the preparation method of the plant-flavored filter stick can include the following steps:
(S1) mixing 4-5 parts by weight of plant raw material powder with aroma, 4-6 parts by weight of smoking agent, 4-6 parts by weight of adhesive and 4-6 parts by weight of water, and making the resultant into a block-shaped wet material;
(S2) squeezing the wet material;
(S3) cutting and separating the squeezed wet material;
(S4) spraying the essence evenly onto the cut and separated wet material to obtain the semi-processed flavored wet material;
(S5) molding the semi-processed plant-flavored filter stick by extrusion molding; and
(S6) drying the semi-processed plant-flavored filter stick to obtain the plant-flavored filter stick.

According to one example of the present disclosure, drying the semi-processed plant-flavored filter stick in the step (S6) can be implemented as follows: at a temperature of 100-110°C, drying the semi-processed plant-flavored filter stick until the water content therein is 8-10% by weight.

According to one example of the present disclosure, in the step (S3), the squeezed wet material can be cut and separated into filamentary materials.

According to one example of the present disclosure, the preparation method of the plant-flavored filter stick can include the following step:
(S8) after spraying the essence onto the cut and separated wet material to form the semi-processed flavored wet material, placing the semi-processed flavored wet material in an airtight environment at 23±2°C and a humidity of 60±5% for a predetermined period of time.

According to some embodiments of the present disclosure, the present disclosure provides a tobacco product, the tobacco product can include a smoking segment, a cooling segment and a filter segment, wherein the smoking segment and the filter segment can be provided at two ends of the cooling segment, respectively. The filter segment can be prepared by the preparation method of a plant-flavored filter stick according to any one of claims 7-9.

The further objects and advantages of the present disclosure will be fully demonstrated by understanding the following descriptions.

These and other objects, characteristics and advantages of the present disclosure will be fully demonstrated by following detailed description.

### Brief Description of Drawings

Fig. 1 shows a stereogram of a tobacco product as described in the present disclosure.
Fig. 2 shows a flow chart of the method for preparing the tobacco product described in the present disclosure.

### Detailed Description of Embodiments

The preferred embodiments described in the following are only examples, and those skilled in the art can think of other obvious variations. The basic principles defined in the following description of the present disclosure can be applied to other embodiments, variation solutions, improvement solutions, equivalent solutions, and other technical solutions that do not depart from the spirit and scope of the present disclosure.

It should be understood by those skilled in the art that in the present disclosure, the terms "vertical", "transverse", "up", "low", "forward", "backward", "left", "right", "upright", "horizontal", "top", "bottom", "inner", "outer" and other directions or positional relationships indicate the directions or positional relationships shown in the drawings, which are only for convenience of describing the present disclosure and simplification of description, and do not indicate or imply that the device or component mentioned must be in a specific direction, or structured or operated in a specific direction, thus the abovementioned terms should not be interpreted as limitations on the present disclosure.

With reference to Fig. 1 to Fig. 2 of the specification, a tobacco product according to the embodiment of the present disclosure will be described in detail below, wherein the tobacco product can be a tobacco product that is heated and burned to form smoke by volatilizing aerosol, or a tobacco product that is heat-not-burn to form smoke by volatilizing aerosol. The present disclosure is not limited in this aspect.

The tobacco product of the present disclosure can include a smoking segment 10, a cooling segment 20 and a filter segment 30. The smoking segment 10 and the filter segment 30 can be respectively installed at two ends of the cooling segment 20, so that the smoking segment 10 can form smoke by volatilizing aerosol, after the smoking segment 10 is heated and the user smokes the filter segment 30.

The cooling segment 20 can reduce the temperature of the smoke formed by volatilization of the heated smoking segment 10 when the user smokes the filter segment 30, so as to prevent the user's mouth from being scalded.

The filter segment 30 can be implemented as a plant-flavored filter stick, wherein the plant-flavored filter stick can be configured as having gas hole passing through both ends of the filter segment 30, and the filter segment 30 can include:
4-5 parts by weight of plant raw material powder with aroma;
4-6 parts by weight of smoking agent;
4-6 parts by weight of adhesive; and
4-6 parts by weight of water.

It is worth mentioning that the plant powder can include but is not limited to cultivated plants and wild plants with aroma. For example, it may include, but is not limited to, tangerine peel, licorice, lavender, basil, mint, rosemary, purple perilla and the like.

More preferably, the filter segment 30 can also include a predetermined amount of essence solidified on the plant-flavored filter stick. The essence can include at least one of water-soluble essence, oil-soluble essence and microencapsulated essence. Specifically, the essence can be implemented as one or more of tangerine peel essence, sweet orange essence, mint essence, jasmine essence, passion fruit essence, amyl acetate, ionone, phenylethyl alcohol, eugenol and perillartine.

Preferably, the solvent of the oil-soluble essence can preferably be medium-chain triglyceride, glycerol triacetate, triethyl citrate and so on, such that the adsorption capacity of the essence is increased.

More preferably, the cooling segment 20 can be implemented as a plant element with a porous structure penetrating through the cooling segment 20. Therefore, after the smoking segment 10 is heated, the aroma emitted by the essence on the plant-flavored filter stick through the holes on the plant element when heated can be mixed in the aerosol formed by volatilization of the smoking segment 10, thereby achieving the uniform diffusion of aroma.

The plant-flavored filter stick itself is composed of fragrant plant raw material powder, and therefore, the plant-flavored filter stick can volatilize sufficient aroma after being heated, so as to make up for the lack of aroma of tobacco products in the prior art.

According to some embodiments of the present disclosure, the present disclosure provides a preparation method of the plant-flavored filter stick, the preparation method of the plant-flavored filter stick can include the following steps:
(S1) mixing 4-5 parts by weight of plant raw material powder with aroma, 4-6 parts by weight of smoking agent, 4-6 parts by weight of adhesive and 4-6 parts by weight of water, and making the mixture into block-shaped wet material;
(S2) squeezing the wet material;
(S3) cutting and separating the squeezed wet material;
(S4) spraying the aroma evenly onto the cut and separated wet material to obtain the semi-processed flavored wet material;
(S5) molding the semi-processed plant-flavored filter stick by extrusion molding; and
(S6) drying the semi-processed plant-flavored filter stick to obtain the plant-flavored filter stick.

Preferably, the step (S1) can be implemented as stirring and mixing for 1 h in a kneading device under the condition of 50 r/min, so as to make a block-shaped wet material to be squeezed.

Preferably, drying the semi-processed plant-flavored filter stick in the step (S6) may be implemented as follows: at a temperature of 100-110°C, drying the semi-processed plant-flavored filter stick until the water content is 8-10% by weight. It is worth mentioning that when the moisture in the plant-flavored filter stick is kept at 8-10% by weight, it can help release the aroma of the plant raw material powder with aroma in the plant-flavored filter stick.

Preferably, the preparation method of the plant-flavored filter stick can include the following step:
(S7) before drying the semi-processed plant-flavored filter stick, cutting the semi-processed plant-flavored filter stick into a predetermined length.

It is worth mentioning that, in the step (S3) of the preparation method of the plant-flavored filter stick, the squeezed wet material can be cut into filaments. In this way, the essence sprayed on the plant-flavored filter stick subsequently can be more uniform.

In addition, in the step (S2), squeezing the wet material can make the formed wet material more compact, which is beneficial for the cut and separated wet material to adsorb more essence.

Preferably, the preparation method of the plant-flavored filter stick can include the following step:
(S8) after spraying the essence onto the cut and separated wet material to form the semi-processed flavored wet material, placing the semi-processed flavored wet material in an airtight environment at 23±2°C and a humidity of 60±5% for a predetermined period of time, so that the semi-processed product of the flavored wet material can fully absorb the sprayed essence.

### Example 1

The block-shaped wet material was made by mixing 4.5 parts by weight of plant raw material powder with aroma, 5 parts by weight of smoking agent, 5 parts by weight of adhesive and 5 parts by weight of water, meanwhile the plant-flavored filter stick was made according to the above-mentioned preparation method, wherein the essence can be peppermint oil to prepare the plant-flavored filter stick.

### Comparative Example 1

The filter stick was made according to the method of prior art. After soaking the filter stick directly in the essence (peppermint oil) for 1 h, the essence on the surface was wiped off to obtain an essence-soaked filter stick.

After the filter sticks in Example 1 and Comparative Example were placed at 22°C and 60% relative humidity for different periods of time, the aroma retention capacity of the two filter sticks was compared. The aroma components in the two samples can be identified by using SPME-GC/MS. GC internal standard method can be used for content determination, in which the chromatographic column can be HP-5 capillary column (30 m×0.32 mm×0.25 µm), with 1-octanol as the internal standard. The specific results are shown in the table below. It can be seen from the following Table 1 that the plant-flavored filter stick of Example 1 has a much greater retention capacity for aroma substances than that of the Comparative Example.

**Table 1**

| Type of filter stick | Menthol content in filter stick for 0 days (mg/g) | Menthol content in filter stick for 10 days (mg/g) | Menthol content in filter stick for 20 days (mg/g) | Menthol content in filter stick for 30 days (mg/g) |
|---|---|---|---|---|
| **Example 1 plant-flavored filter stick** | 25.6 | 23.8 | 20.7 | 19.3 |
| **Comparative** | 24.4 | 19.3 | 14.5 | 10.8 |
| **Example filter stick** | | | | |

It is worth mentioning that when making the plant-flavored filter stick, the present disclosure adopts the method of spraying first and then extruding, so that the sprayed essence can be fully mixed with the wet material. After extrusion, the channels through which the essence is emitted can be more compact, which can delay the preservation time of the essence.

Those skilled in the art should understand that the embodiments of the present disclosure shown in the above description are only examples and do not limit the present disclosure. The purpose of the present disclosure has been fully and effectively achieved. The functions and structural principles of the present disclosure have been shown and described in the examples, and any deformation or modification can be made to the embodiments of the present disclosure without departing from the principles.

### Industrial Applicability

The present disclosure provides a tobacco product and a plant-flavored filter stick thereof, and a preparation method therefor, wherein the plant-flavored filter stick can be implemented as a filter stick having a gas hole passing through two ends of the filter segment, and the plant-flavored filter stick includes: 4-5 parts by weight of plant raw material powder with aroma, 4-6 parts by weight of smoking agent, 4-6 parts by weight of adhesive and 4-6 parts by weight of water, which can achieve the flavor-enhancing of tobacco products. The plant-flavored filter stick uses the natural aroma of the filter stick itself and the aroma emitted by the flavor-enhancing substance added to the filter stick to enhance the aroma of tobacco products. In addition, the plant-flavored filter stick can avoid the loss and thermal degradation (the escape and pyrolysis) of flavor-enhancing substances during storage and smoking of tobacco products.

In addition, it can be understood that a tobacco product and a plant-flavored filter stick thereof, and a preparation method therefor of the present disclosure are reproducible and can be applied in various applications. For example, the preparation method of a plant-flavored filter stick of the present disclosure can be applied to produce a plant-flavored filter stick.

## Claims

1. A plant-flavored filter stick, **characterized in that** the plant-flavored filter stick is configured to have gas holes passing through two ends of the plant-flavored filter stick, and the plant-flavored filter stick comprises:
4-5 parts by weight of a plant raw material powder with aroma;
4-6 parts by weight of a smoking agent;
4-6 parts by weight of an adhesive; and
4-6 parts by weight of water.

2. The plant-flavored filter stick according to claim 1, wherein the plant raw material powder comprises cultivated plants and wild plants with aroma.

3. The plant-flavored filter stick according to claim 1 or 2, wherein the plant-flavored filter stick comprises a predetermined amount of an essence solidified on the plant-flavored filter stick.

4. The plant-flavored filter stick according to claim 3, wherein the essence comprises at least one of water-soluble essences, oil-soluble essences and microencapsulated essences.

5. The plant-flavored filter stick according to claim 4, wherein a solvent of the oil-soluble essences is preferably selected from the group consisting of medium-chain triglyceride, glycerol triacetate and triethyl citrate.

6. A tobacco product, **characterized in that** the tobacco product comprises a smoking segment, a cooling segment and a filter segment, wherein the smoking segment and the filter segment are respectively provided at two ends of the cooling segment, and the filter segment is configured as the plant-flavored filter stick according to any one of claims 1-5.

7. The tobacco product according to claim 6, wherein the cooling segment is configured as a plant element with a porous structure penetrating through the cooling segment.

8. A preparation method of a plant-flavored filter stick, **characterized in that** the preparation method of the plant-flavored filter stick comprises following steps:
(S1) mixing 4-5 parts by weight of a plant raw material powder with aroma, 4-6 parts by weight of a smoking agent, 4-6 parts by weight of an adhesive and 4-6 parts by weight of water, and making a resultant into a block-shaped wet material;
(S2) squeezing the wet material;
(S3) cutting and separating a squeezed wet material;
(S4) spraying an essence evenly onto a cut and separated wet material to obtain a semi-processed flavored wet material;
(S5) molding a semi-processed plant-flavored filter stick by extrusion molding; and
(S6) drying the semi-processed plant-flavored filter stick to obtain the plant-flavored filter stick.

9. The preparation method of the plant-flavored filter stick according to claim 8, wherein the drying the semi-processed plant-flavored filter stick in the step (S6) is implemented as follows: at a temperature of 100-110°C, drying the semi-processed plant-flavored filter stick until a water content is 8-10% by weight.

10. The preparation method of the plant-flavored filter stick according to claim 8 or 9, wherein in the step (S3), the squeezed wet material is cut and separated into filamentary materials.

11. The preparation method of the plant-flavored filter stick according to any one of claims 8-10, wherein the preparation method of the plant-flavored filter stick comprises a following step:
(S8) after spraying the essence onto the cut and separated wet material to form the semi-processed flavored wet material, placing the semi-processed flavored wet material in an airtight environment at 23±2°C and a humidity of 60±5% for a predetermined period of time.

12. A tobacco product, **characterized in that** the tobacco product comprises a smoking segment, a cooling segment and a filter segment, and the smoking segment and the filter segment are respectively provided at two ends of the cooling segment, wherein the filter segment is configured to be made by the preparation method of the plant-flavored filter stick according to any one of claims 8-11.
